

## UNITED STATES PATENT OFFICE.

ANTOINE REGNOUF DE VAINS, OF MIRIBEL, FRANCE.

## MANUFACTURE OF CELLULOSE.

No Drawing.

Application filed October 19, 1923. Serial No. 669,623.

*To all whom it may concern:*

Be it known that I, ANTOINE REGNOUF DE VAINS, a citizen of the Republic of France, residing at 10 Rue Henri Grosbon, Miribel, 5 Ain, France, have invented new and useful Improvements in the Manufacture of Cellulose, of which the following is a specification.

The present invention relates to a process 10 for neutralizing the acids set free by the chlorination of cellulosic material treated with chlorine with a view to bleaching and for dissolving the chlorinated products, such as ketonic chlorides, resulting from this 15 treatment.

The inventor has already proposed a process of this kind which consists in treating the chlorinated cellulosic material (paper-pulp) with bases of the alkali earth metals 20 or with salts of the alkali earth metals whose acid is weaker than hydrochloric acid. This process is subject to the drawback that it introduces into the paper-pulp after chlorination a considerable quantity of 25 bases or salts of the alkali earth metals. It has been found impossible in practice to obtain an exact neutralization of the products to be destroyed and, it is necessary to use an excess of bases or salts of the alkali 30 earth metals, which excess remains in the pulp and prevents it being properly bleached. This process is described in French Patent No. 550,925, granted May 3, 1922.

On the other hand, the inventor has also proposed another process (U. S. Patent No. 1,455,495, granted February 13, 1923), which provides for the solution of the chlorinated derivatives, resulting from the treatment of ligno- and pecto-cellulose by chlorine, by 40 means of soda residuary liquors, which have already served to lixiviate cellulosic material. This process is subject to the serious drawback that it consumes a considerable quantity of these liquors and, owing to this circumstance, the soda element which they 45 contain is entirely lost.

The present invention enables these drawbacks to be overcome in a satisfactory manner and it consists in combining the two known processes, that is to say: in treating the chlorinated ligno- and pecto-cellulose with a restricted quantity of bases or salts

of the alkali earth metals so as to obtain an approximate neutralization of the acids set 55 free by the chlorination; in washing the pulp which has been neutralized in this manner and in treating it with the residuary soda liquors or any other sodium hydroxide solution, such as a solution of sodium hydroxide, of sodium carbonate, sodium sulphite and the like, with a view to rendering soluble the derivatives formed during the chlorination, which derivatives can then 60 easily be eliminated by washing with water; the chlorinated products are thus eliminated after a preliminary stage or neutralizing stage, by treating the pulp with bases or salts of the alkali earth metals and the second stage or stage of solution of the chlorinated products, is effected with the help of 65 soda reagents. The technical effect of the present invention results from the statements given above, and the economic effect 70 consists in the fact that a great saving in soda reagents is effected as compared with the known process, said reagents being replaced by reagents of the group of alkali 75 earth metals which are less expensive and which, however, perform the same work. Furthermore, the cellulosic material obtained 80 does not contain an excess of alkali earth metals which are prejudicial to the whiteness of the pulp.

When carrying out the invention in practice, the chlorinated pulp is fed continuously to a malaxating apparatus of any suitable form, having either a vertical shaft, a horizontal shaft or being provided with baffles. At the same time, there is continuously fed 90 to the same malaxating apparatus, either a milk of lime or a milk of calcium carbonate, or salt of any other alkali earth metal. The pulp is then washed by any known means in order to extract the alkali earth metal chlorides formed which, if these precautions 95 were not taken, would react with the soda in the subsequent alkaline treatment and would consequently consume a large quantity of valuable reagent. The pulp obtained 100 is then treated with an alkaline base such as caustic soda, caustic potash or ammonia or, with a salt of one of these bases formed by an acid weaker than hydrochloric acid, such as sodium carbonate, sodium sulphite and the 105 like. The solution of the chlorinated deriva-

tives is then very economically effected by lixiviation with water and the pulp is then finally bleached by the usual process.

Any residuary liquors, whether of soda or alkali earth metals, having already served for the lixiviation of cellulose material in other operations, may be used as reagents.

I claim:

1. Process for neutralizing the acids set free by the chlorination of cellulosic material and for dissolving out the chlorinated derivatives, consisting in neutralizing, by means of a compound of the alkaline earth metals, the chlorinated cellulose and in rendering soluble, by means of an alkaline compound, the chlorinated derivatives formed during chlorination.

2. A process, as in claim 1, in which the cellulosic pulp is washed after the operation of neutralization.

3. A process as in claim 1, in which the chlorinated derivatives are washed out after they have been rendered soluble.

4. A process as in claim 1, in which the chlorinated derivatives are washed out after they have been rendered soluble and the pulp has been neutralized.

5. A process as in claim 1, in which the compound of an alkaline earth metal consists of a residuary liquor of the alkali earth metal group, which has already served for lixiviating cellulosic material during other operations.

6. A process as in claim 1, in which the alkaline compound consists of an alkaline residuary liquor having already served for lixiviating cellulosic material during other operations.

ANTOINE REGNOUF DE VAINS.